

## [54] PHOTOGRAPHIC COLOUR MATERIAL

[75] Inventors: **Hector Alfons Vanden Eynde, Edegem; Raphael Karel Van Poucke, Berchem; Arthur Henri De Cat, Mortsel; Gaston Jacob Benoy, Edegem**, all of Belgium

[73] Assignee: **Gevaert-AGFA N.V., Mortsel, Belgium**

[22] Filed: **Feb. 8, 1971**

[21] Appl. No.: **113,647**

## [30] Foreign Application Priority Data

Feb. 24, 1970 Belgium ..... 8839

[52] U.S. Cl. .... **96/55, 96/56.1, 96/74, 96/100, 260/618**

[51] Int. Cl. .... **G03c 7/00**

[58] Field of Search ..... **96/100, 9, 74**

## [56] References Cited

## UNITED STATES PATENTS

|           |         |                     |        |
|-----------|---------|---------------------|--------|
| 3,005,709 | 10/1961 | Coles .....         | 96/100 |
| 3,013,879 | 12/1961 | de Ramaix .....     | 96/9   |
| 3,244,520 | 4/1966  | Schulte et al. .... | 96/100 |

Primary Examiner—J. Travis Brown

Attorney—Brufsky, Staas, Breiner & Halsey

## [57] ABSTRACT

Light-sensitive silver halide color emulsions are described which comprise a cyan-forming color coupler of the formula:



wherein:

Z represents the atoms necessary to close a fused-on benzene or tetrahydrobenzene ring,

Y represents hydrogen or a substituent conferring to the color coupler a 2-equivalent character,

R<sub>1</sub> represents a straight-chain C<sub>1</sub>–C<sub>5</sub> alkyl group or an aryl group with electron-withdrawing substituent,

R<sub>2</sub> represents a straight-chain C<sub>1</sub>–C<sub>5</sub> alkyl group, or R<sub>2</sub> together with R<sub>1</sub> represents the atoms necessary to close a cycloaliphatic ring, and

R<sub>3</sub> stands for a diffusion-fast making straight-chain acyclic aliphatic hydrocarbon group comprising from 10 to about 20 C-atoms or for a residue substituted by a diffusion-fast making acyclic aliphatic hydrocarbon group having from 10 to about 20 C-atoms, or R<sub>3</sub> together with R<sub>1</sub> represents the atoms necessary to complete a diffusion fast making cycloaliphatic hydrocarbon group which comprises in the ring or together with the C-atoms of an alkyl substituent on the ring at least 12 C-atoms. Upon exposure and color development, cyan dyestuff images are formed in the described emulsions which have favorable spectral properties and a high stability against heat.

9 Claims, No Drawings

## PHOTOGRAPHIC COLOUR MATERIAL

This invention relates to novel cyan forming colour couplers, to the use thereof in the production of photographic colour images and to photographic material containing such colour couplers.

It is known that for the production of a photographic colour image in a light-sensitive silver halide layer, the exposed silver halide is developed to a silver image by means of an aromatic primary amino compound in the presence of a colour coupler which reacts with the oxidized developing substance to form a dyestuff on the areas corresponding to the silver image.

In the subtractive three-colour photography a light-sensitive photographic colour material is used containing a red-sensitized, a green-sensitized and a blue-sensitive silver halide emulsion layer wherein on colour development, by the use of appropriate colour couplers, a cyan, magenta and yellow dyestuff image are formed respectively.

The colour couplers may be added directly to the developer solution or they can be incorporated in the photographic material. In the latter case, it is required that the colour couplers do not wander or diffuse through the emulsion from their original site. For this purpose the colour couplers are usually provided in their molecule with one or more ballast groups, e.g. a long chain aliphatic group such as an alkyl group containing from 12 to 20 C-atoms in straight line. This ballast group imparts to the molecule a hydrophobic character and holds the component firmly in its original site.

Various methods have been described to incorporate these non-diffusing colour couplers into hydrophilic colloid compositions.

A method commonly employed to incorporate the non-diffusing colour couplers into hydrophilic colloid compositions such as a gelatino silver halide emulsion is to provide in the molecule of said couplers in addition to the ballasting group one or more salt-forming groups more particularly carboxy and/or sulpho groups so that the couplers can be dissolved in the hydrophilic colloid composition in the form of their soluble alkali metal salts.

Alternate methods of incorporating non-diffusing colour couplers in hydrophilic colloid compositions make use of dispersion techniques.

According to one such method, e.g. as described in German Patent Specification 1,127,714 water-insoluble colour couplers are dissolved in low-boiling substantially water-immiscible solvents such as ethyl acetate, methylene chloride, chloroform, etc. whereupon the solution formed is dispersed in extremely fine droplets in the presence of a wetting agent into the hydrophilic colloid medium after which the solvent is removed by evaporation, leaving behind a dispersion of colour coupler distributed throughout the hydrophilic colloid composition.

Another process for dispersing non-diffusing colour couplers in photographic hydrophilic colloid compositions is described in U.S. Pat. No. 2,322,027. According to this process a colour coupler is dissolved in a high-boiling oily solvent such as tricresyl phosphate and di-n-butyl-phthalate whereupon the resulting solution is dispersed in the form of extremely fine droplets in the hydrophilic colloid composition, the oily solvent being left in the said composition.

In preparing silver halide emulsions comprising non-diffusing colour couplers by the use of dispersion techniques various difficulties are encountered. Indeed, colour couplers that are intended to be incorporated into photographic colloid media from solutions in low-boiling or high-boiling organic solvents should have a sufficient solubility in said solvents and be homogeneously distributed through the said colloid media before as well as after coating to form a hydrophilic colloid layer of a photographic multilayer colour material so that no crystallization of the colour coupler occurs. This condition limits the number of colour couplers suitable for such applications.

In U.S. Pat. No. 3,005,709 1-hydroxy-2-naphthamide colour couplers for cyan have been disclosed in which the amide group is derived from highly branched tertiary alkyl amines. In order to be perfectly non-diffusible in hydrophilic colloid media highly branched tertiary alkyl amines sold under the trade name "Primene SM-T" by the Rohm and Haas Company, Philadelphia, Pennsylvania, U.S.A. are used in the preparation of the 1-hydroxy-2-naphthamide colour couplers. Though these non-diffusing cyan-forming colour couplers have high solubility in oily type organic solvents and high resistance to crystallization so that they are very suitable for being incorporated into photographic colloid media by means of the above dispersion techniques, they show the disadvantage of yielding upon colour development with an aromatic primary amino colour developing agent dyes with unrepeatable spectral and sensitometric characteristics and too low a maximum density.

It is an object of the present invention to provide cyan-forming colour couplers which do not diffuse from one hydrophilic colloid layer into another when incorporated in a multilayer colour material.

A further object of the present invention is to provide 1-hydroxy-2-naphthamide cyan-forming colour couplers in which the amide group is derived from amines with tertiary  $\alpha$ -carbon atoms which yield upon colour development dyes with reproducible spectral and sensitometric characteristics.

Another object of the present invention is to provide cyan forming colour couplers which have the same favourable high solubility in organic solvents such as low-boiling or high-boiling sparingly water-miscible solvents as the colour couplers of the above United States Patent Specification.

Other objects will appear from the description below.

These objects are accomplished by the use of cyan forming colour couplers corresponding to the following general formula :



wherein :

Z represents the atoms necessary to close a fused-on benzene or tetrahydrobenzene ring,

Y represents hydrogen or a substituent which confers to the colour coupler a 2-equivalent character such as halogen e.g. chlorine and bromine, sulpho in acid or salt form, azo such as phenylazo and substi-

tuted phenylazo, the group  $-\text{S}-\text{R}$  wherein  $\text{R}$  stands for alkyl, aryl or a heterocycle, etc.

$\text{R}_1$  represents a straight-chain  $\text{C}_1\text{--C}_5$  alkyl such as methyl, ethyl, and propyl or an aryl group with electron-withdrawing substituent for example m-chlorophenyl,

$\text{R}_2$  represents a straight-chain  $\text{C}_1\text{--C}_5$  alkyl such as methyl, ethyl and propyl, or

$\text{R}_1$  together with  $\text{R}_2$  represent the atoms necessary to close a cyclo-aliphatic ring e.g., cyclohexyl, and

$\text{R}_3$  represents a straight-chain acyclic aliphatic hydrocarbon group with from 10 to about 20 C-atoms which renders the molecule fast to diffusion in photographic hydrophilic colloid media or a residue comprising a diffusion-fast making acyclic aliphatic hydrocarbon group such as the residues  $-\text{X}_1\text{--D}$  and  $-\text{CH}_2\text{--X}_2\text{--D}$  wherein D stands for an acyclic aliphatic hydrocarbon group with from 10 to about 20 C-atoms,  $\text{X}_1$  stands for  $-\text{COO--}$ ,  $-\text{CON}(\text{R}_4)\text{--}$ ,



$\text{R}_4$  being hydrogen or  $\text{C}_1\text{--C}_5$  alkyl and  $\text{Y}_1$  being a chemical bond, oxygen, sulphur, sulphonyl,  $\text{NHCO}$ ,  $\text{CONH}$ ,  $\text{NHSO}_2$  or  $\text{SO}_2\text{NH}$ , and  $\text{X}_2$  stands for  $-\text{N}(\text{R}-\text{4})\text{--}$ , sulphur,  $-\text{CON}(\text{R}_4)\text{--}$ ,  $-\text{COO--}$ ,



,  $\text{R}_4$  and  $\text{Y}_1$  having the same significance as above, or  $\text{R}_3$  together with  $\text{R}_1$  represent the atoms necessary to complete a diffusion fast-making cycloaliphatic hydrocarbon group which comprises in the ring or together with the C-atoms of an alkyl substituent on the ring at least 12 C-atoms.

The novel cyan-forming colour couplers according to the present invention were not only found to be very suitable for being incorporated into photographic hydrophilic colloid media by means of dispersion techniques in that they have a high solubility in the organic solvents used therefor but it was also found that they yield dyes which possess besides favourable spectral properties an excellent stability against heat.

The following compounds are representative colour couplers corresponding to the above general formula :



3.



10



15



20



25



30



35



40



55



60





Colour coupler 4 was prepared in a similar way as colour coupler 1 from phenyl 5,6,7,8-tetrahydro-1-hydroxy-4-chloro-2-naphthoate and  $\alpha,\alpha$ -dimethylhexadecylamine.

Yield : 65 percent.

Melting point : 34°C.

Preparation 5 : Colour coupler 5

Colour coupler 5 was prepared in a similar way as colour coupler 1 from phenyl 1-hydroxy-4-chloro-2-naphthoate and  $\alpha,\alpha$ -diethylhexadecylamine.

Yield : 91 percent.

The  $\alpha,\alpha$ -diethylhexadecylamine was prepared in a similar way as  $\alpha,\alpha$ -dimethylhexadecylamine from  $\alpha,\alpha$ -diethylhexadecylalcohol.

Yield : 76 percent.

Boiling point : 135°-140°C/0.2 mm.

The  $\alpha,\alpha$ -diethylhexadecylalcohol was prepared in a similar way as  $\alpha,\alpha$ -dimethylhexadecylalcohol from ethyl iodide, magnesium and methyl palmitate.

Yield : 97 percent.

Melting point : 33°C.

Preparation 6 : Colour Coupler 6

Colour coupler 6 was prepared in a similar way as colour coupler 1 from phenyl 1-hydroxy-4-chloro-2-naphthoate and  $\alpha,\alpha$ -di-n-propyloctadecylamine.

Yield : 80 percent.

The  $\alpha,\alpha$ -di-n-propyloctadecylamine was prepared in a similar way as  $\alpha,\alpha$ -dimethylhexadecylamine from  $\alpha,\alpha$ -di-n-propyloctadecyl-alcohol.

Yield : 60 percent.

Boiling point : 155°-160°C/0.15 mm.

The  $\alpha,\alpha$ -di-n-propyloctadecylalcohol was prepared in a similar way as  $\alpha,\alpha$ -dimethylhexadecylalcohol from n-propyl iodide, magnesium and methyl stearate.

Yield : 95 percent.

Melting point : 30°C.

Preparation 7 : Colour coupler 7

a. Methyl  $\alpha$ -(1-hydroxy-4-chloro-2-naphthoylamino)isobutyrate 95.5 g of methyl  $\alpha$ -aminoisobutyrate, prepared as described in *Tetrahedron* 11, 43-44 (1960), starting from  $\alpha$ -aminoisobutyric acid which is commercially available from the firm Dr.Th.Schuchardt Munich, W.Germany, and 243.5 g of phenyl 1-hydroxy-4-chloro-2-naphthoate were heated with stirring on an oil bath for 2 hours at 130°C and then for 2 hours at 155°-160°C.

The reaction mixture was recrystallized from 1 litre of cyclohexane.

Yield : 172.5 g (66 percent).

Melting point : 159°-160°C.

b.  $\alpha$ -(1-hydroxy-4-chloro-2-naphthoylamino)isobutyric acid

160.75 g of the above isobutyrate in 1 litre of N sodium hydroxide were heated with stirring to the boiling temperature. After approximately 10 minutes a solution was obtained which was then cooled in an ice-bath and to which was added dropwise with stirring 100 ml of concentrated hydrochloric acid.

The precipitate formed was filtered by suction, washed with water and while moist recrystallized from 350 ml of methanol.

Yield : 149 g (97 percent).

Melting point : 189°C.

c. N-dodecyloxypropyl- $\alpha$ -(1-hydroxy-4-chloro-2-naphthoylamino) isobutyramide

15.4 g of the above isobutyric acid were dissolved in 50 ml of anhydrous acetonitrile whereupon 12.2 g of

dodecyloxypropylamine, commercially available from the firm Dr.Th.Schuchardt, Munich, W.Germany, were added with stirring. At a temperature of approximately 20°C, 11.3 g of dicyclohexylcarbodiimide, which is also commercially available from the above firm, were added dropwise whereby the temperature of the reaction mixture rose to 42°C. Stirring was continued for 1 hour whereupon the mixture was refluxed for 10 minutes. The dicyclohexylurea formed was filtered off and the product that crystallized in the filtrate was isolated and washed with acetonitrile.

Yield : 23 g (86.5 percent).

Melting point : 67°C.

Preparation 8 : Colour coupler 8

15 N-methyl-N-octadecyl- $\alpha$ -(1-hydroxy-4-chloro-2-naphthoylamino)-isobutyramide was prepared in a similar way as colour coupler 7 starting from N-methyl-N-octadecylamine,  $\alpha$ -(1-hydroxy-4-chloro-2-naphthoylamino) isobutyric acid and dicyclohexylcarbodiimide.

Yield : 75 percent.

Melting point : 70°-72°C.

Preparation 9 : Colour coupler 9

a. ethyl  $\beta$ -(1-hydroxy-4-chloro-2-naphthoylamino)-isovalerate 65 g of ethyl  $\beta$ -amino-isovalerate, prepared as described in Ann. 661, 111 (1963), and 134 g of phenyl 1-hydroxy-4-chloro-2-naphthoate were heated with stirring on an oil bath for 2 hours at 135°-140°C and then for 2 hours at 165°C.

30 The phenol formed was distilled off under reduced pressure and the residue was recrystallized from 300 ml of ethanol.

Yield : 119 g (76 percent).

Melting point : 103°C.

35 b.  $\beta$ -(1-hydroxy-4-chloro-2-naphthoylamino)-isovaleric acid

116 g of the above isovalerate in 700 ml of N sodium hydroxide were heated with stirring at the boiling temperature whereby a solution formed. Heating was continued for 10 min. and the solution was then cooled in an ice-bath. Concentrated hydrochloric acid was added dropwise and the precipitate formed was isolated and washed with water. The product was stirred in 100 ml of methanol, filtered by suction and recrystallized from 320 ml of acetonitrile.

Yield : 82 g (76.5 percent).

Melting point : 172°-174°C.

c. N-(o-hexadecyloxyphenyl)  $\beta$ -(1-hydroxy-4-chloro-2-naphthoylamino)isovaleramide

50 17.7 g of the above isovaleric acid were dissolved in 60 ml of anhydrous acetonitrile and 18.8 g of o-hexadecyloxyaniline were added with stirring. 13.2 g of dicyclohexylcarbodiimide were added dropwise at room-temperature whereby an exothermic reaction started; stirring was continued for 1 hour whereupon the mixture was refluxed for 10 minutes. The dicyclohexylurea formed was filtered off and to the hot filtrate methylene chloride was added in such an amount that the oily precipitate dissolved. The white product that crystallized was filtered off by suction, washed with methanol and dried.

Yield : 28.3 g (81 percent).

Melting point : 90°C.

Preparation 10 : Colour coupler 10

N-methyl-N-octadecyl  $\beta$ -(1-hydroxy-4-chloro-2-naphthoylamino) isovaleramide was prepared in a similar way as colour coupler 9 from N-methyl-N-

octadecylamine,  $\beta$ -(1-hydroxy-4-chloro-2-naphthoyl-amino)-isovaleric acid and dicyclohexylcarbodiimide.

Yield : 82.5 percent.

Melting point : 57°C.

Preparation 11 : Colour coupler 11

This colour coupler was prepared in a similar way as colour coupler 1 from phenyl 1-hydroxy-4-chloro-2-naphthoate and  $\alpha,\alpha$ -diethyldocosylamine.

Yield : 85 percent.

Melting point : 44°C.

The  $\alpha,\alpha$ -diethyldocosylamine was prepared in a similar way as m-dodecyloxy- $\alpha$ -methyl- $\alpha$ -ethylbenzylamine and preparation of which is given hereinafter, from  $\alpha,\alpha$ -diethyldocosylalcohol.

Yield : 82 percent.

Melting point : 26°C.

The  $\alpha,\alpha$ -diethyldocosylalcohol was prepared in a similar way as  $\alpha,\alpha$ -dimethylhexadecylalcohol ethyl iodide, magnesium, and methylbehenate.

Yield : 97 percent.

Melting point : 52°C.

Methyl behenate was prepared from behenic acid, sulphurous oxychloride and methyl alcohol.

Yield : 96 percent.

Melting point : 51°-52°C.

Preparation 12 : Colour coupler 12

This colour coupler was prepared in a similar way as colour coupler 9 from  $\gamma$ -lauryloxy-propylamine,  $\beta$ -(1-hydroxy-4-chloro-2-naphthoylamino)-isovaleric acid and dicyclohexylcarbodiimide.

Yield : 57 percent.

Preparation 13 : Colour coupler 13

This colour coupler was prepared in a similar way as colour coupler 1 from phenyl 1-hydroxy-4-chloro-2-naphthoate and  $\alpha$ -methyl- $\alpha$ -ethyl-octadecylamine.

Yield : 83 percent.

Melting point : 55°C.

The  $\alpha$ -methyl- $\alpha$ -ethyloctadecylamine was prepared in a similar way as  $\alpha,\alpha$ -dimethylhexadecylamine from  $\alpha$ -methyl- $\alpha$ -ethyloctadecyl alcohol.

Yield : 50 percent.

The  $\alpha$ -methyl- $\alpha$ -ethyloctadecylalcohol was prepared as follows :

To the Grignard solution prepared in a similar way as in preparation 1a) from 60 g of magnesium, 390 g of ethyl iodide and 875 ml diethylether, a solution of 562 g of methyl heptadecyl ketone was added in such a way that refluxing continued due to the exothermic reaction. The mixture was further refluxed for 2 hours on a hot water bath whereupon the reaction mixture was poured with stirring into a solution of 500 g of ammonium chloride in 5 litres of ice-water. The ether solution was washed with water and dried. The ether was then removed by evaporation leaving a residue of  $\alpha$ -methyl- $\alpha$ -ethyloctadecylalcohol.

Yield : 94 percent.

Preparation 14 : Colour coupler 14

a. m-dodecyloxy- $\alpha$ -methyl- $\alpha$ -ethylbenzylalcohol

To the Grignard solution prepared in a similar way as in preparation 1a) from 30 g of magnesium, 195 g of ethyl iodide and 300 ml of diethylether, a solution of 304 g of m-dodecyloxyacetophenone in 1250 ml of diethylether was added in such a way that refluxing continued due to the exothermic reaction. When all was added, refluxing was continued for 2 hours, whereupon the mixture was poured with stirring into a solution of 250 g of ammonium chloride in 2.5 litres of ice-water.

The ether layer was washed with water and dried. The ether was removed by evaporation leaving a residue of m-dodecyloxy- $\alpha$ -methyl- $\alpha$ -ethylbenzylalcohol.

Yield : 96.5 percent.

b. m-dodecyloxy- $\alpha$ -methyl- $\alpha$ -ethylbenzylamine

267.5 g of the above alcohol and 98 g of sodium cyanide were stirred at 40°C in 600 ml of n-dibutylether. Then 240 ml of 95 percent sulphuric acid was added dropwise in such a way that the temperature is kept at 40°-45°C by the exothermic reaction. Stirring was then continued for 2 hours on a water-bath of 50°C.

600 ml of n-butanol were added to the reaction mixture whereupon the mixture was refluxed for 2 hours with stirring. The mixture was made strongly alkaline

15 by addition of 5N sodium hydroxide whereupon the organic layer was separated, washed with water and concentrated by evaporation till dry. The crude reaction product was purified by turning into the oxalate in a mixture of diethylether and methanol. The oxalate was filtered off whereupon by addition of alkali in isopropylether the m-dodecyloxy- $\alpha$ -methyl- $\alpha$ -ethylbenzylamine was set free.

Yield : 45 percent.

Melting point : 122°C.

c. Colour coupler 14

This colour coupler was prepared in a similar way as colour coupler 1 from phenyl 1-hydroxy-4-chloro-2-naphthoate and m-dodecyloxy- $\alpha$ -methyl- $\alpha$ -ethylbenzylamine.

30 Yield : 82 percent.

Preparation 15: Colour coupler 15

a.  $\beta$ -dodecylthio- $\alpha,\alpha$ -dimethylpropionic acid

35 157 g of chloropivalic acid, 232 g of dodecylmercaptan and 151 g of 85 percent potassium hydroxide were refluxed for 3 hours with stirring in 1 litre of ethylene glycol monomethylether. The mixture was then poured into a mixture of 1 litre of ice-water and 500 ml of concentrated hydrochloric acid. The product formed was

40 extracted with diethylether and washed acid free with water. The ether layer was dried and concentrated by evaporation till dry.

The crude product was subjected to fractional distillation.

45 Yield : 230 g (66 percent).

Boiling point : 177°-178°C/0.3 mm

b.  $\beta$ -dodecylthio- $\alpha,\alpha$ -dimethylethylamine

50 75 g of the above compound and 250 ml of dry benzene were stirred and 227 ml of 95 percent sulphuric acid were added. The mixture was heated to 45°C whereupon 18 g of sodium azide were added portionwise in 1 hour so that the temperature was kept at 45°-50°C by the exothermic reaction. The mixture was further heated on a water bath of 50°C until all gas evolution ceased.

55 The underlying acid layer was separated and poured with stirring into 1 litre of ice-water. The white precipitate was filtered off and washed with water. The product was set free from its sulphate form by addition of aqueous alkali in methylene chloride. The methylene chloride layer was freed from alkali by washing with water, dried and concentrated by evaporation till dry.

The crude product was recrystallized from cyclohexan.

60 Yield : 40 g (59 percent).

Melting point : 86°C.

c. Colour coupler 15



organic solvents employed, is intimately mixed with the said coating composition of the light-sensitive silver halide emulsion layer or other water-permeable layer just before coating.

For more details about particularly suitable techniques that may be employed for incorporating the colour couplers of the invention into a hydrophilic colloid layer of a photographic material there can be referred to e.g., U.S. Pat. Nos. 2,269,158 - 2,284,887 - 2,304,939 - 2,304,940 and 2,322,027, United Kingdom Pat. Nos. 791,219 - 1,098,594 - 1,099,414 - 1,099,415 - 1,099,416 and 1,099,417, French Pat. No. 1,555,663, Belgian Pat. No. 722,026, German Pat. No. 1,127,714 and to United Kingdom Pat. application No. 14,763/69.

The couplers according to the invention may be used in conjunction with various kinds of photographic emulsions. Various silver salts may be used as the sensitive salt such as silver bromide, silver iodide, silver chloride or mixed silver halides such as silver chlorobromide, silver bromoiodide and silver chlorobromiodide. The couplers can be used in emulsions of the mixed packet type as described in U.S. Pat. No. 2,698,794 or emulsions of the mixed grain type as described in U.S. Pat. No. 2,592,243. The colour couplers can be used with emulsions wherein latent images are formed predominantly on the surface of the silver halide crystal, or with emulsions wherein latent images are formed predominantly inside the silver halide crystal.

The hydrophilic colloid used as the vehicle for the silver halide may be, for example, gelatin, colloidal albumin, zein, casein, a cellulose derivative, a synthetic hydrophilic colloid such as polyvinyl alcohol, poly-N-vinyl pyrrolidone, etc. If desired, compatible mixtures of two or more of these colloids may be employed for dispersing the silver halide.

The light-sensitive silver halide emulsions of use in the preparation of a photographic material according to the present invention may be chemically as well as optically sensitized. They may be chemically sensitized by effecting the ripening in the presence of small amounts of sulphur containing compounds such as allyl thiocyanate, allyl thiourea, sodium thiosulphate, etc. The emulsions may also be sensitized by means of reductors for instance tin compounds as described in French Pat. No. 1,146,955 and in Belgian Pat. No. 568,687, imino-amino methane sulphonic acid compounds as described in United Kingdom Pat. No. 789,823 and small amounts of noble metal compounds such as gold, platinum, palladium, iridium, ruthenium and rhodium compounds. They may be optically sensitized by means of cyanine and merocyanine dyes.

The said emulsions may also comprise compounds which sensitize the emulsions by development acceleration for example compounds of the polyoxyalkylene type such as alkylene oxide condensation products as described among others in U.S. Pat. Nos. 2,531,832 - 2,533,990 - 3,210,191 and 3,158,484, in United Kingdom Pat. Nos. 920,637 and 991,608 and in Belgian Pat. No. 648,710 and onium derivatives of amino-N-oxides as described in United Kingdom Pat. No. 1,121,696.

Further, the emulsions may comprise stabilizers e.g. heterocyclic nitrogen-containing thioxo compounds such as benzothiazoline-2-thione and 1-phenyl-2-tetrazoline-5-thione and compounds of the hydroxytriazolopyrimidine type. They can also be stabilized with

mercury compounds such as the mercury compounds described in Belgian Pat. No. 524,121 - 677,337 and 707,386 and in U.S. Pat. No. 3,179,520.

The light-sensitive emulsions may also comprise all other kinds of ingredients such as plasticizers, hardening agents, wetting agents, etc.

The non-diffusing cyan colour formers described in the present invention are usually incorporated into the red-sensitized silver halide emulsion for forming one of the differently sensitized silver halide emulsion layers of a photographic multilayer colour material. Such photographic multilayer colour material usually comprises a support, a red-sensitized silver halide emulsion layer with a cyan colour former, a green-sensitized silver halide emulsion layer with a magenta colour former and a blue-sensitive silver halide emulsion layer with a yellow colour former.

The emulsions can be coated on a wide variety of photographic emulsion supports. Typical supports include cellulose ester film, polyvinylacetal film, polystyrene film, polyethylene terephthalate film and related films or resinous materials, as well as paper and glass.

For the production of photographic colour images according to the present invention an exposed silver halide emulsion layer is developed with an aromatic primary amino developing substance in the presence of a colour coupler according to the present invention. All colour developing agents capable of forming azomethine dyes can be utilised as developers. Suitable developing agents are aromatic compounds such as p-phenylene diamine and derivatives for example N,N-dialkyl-p-phenylene diamines such as N,N-diethyl-p-phenylene diamine, N,N-dialkyl-N'-sulphomethyl-p-phenylene diamines, and N,N-dialkyl-N'-carboxymethyl-p-phenylene diamines.

The following examples illustrate the present invention.

#### EXAMPLE 1

40 A 5 percent aqueous solution of gelatin having dispersed therein per litre 50 g of colour coupler 7, was prepared by dispersing by means of a high speed stirrer a solution of 1 part by weight of colour coupler in 3 parts by volume of ethyl acetate into the aqueous gelatin at 55°C in the presence of sodium dodecyl benzene sulphonate as dispersing agent followed by removal of the ethyl acetate by evaporation under reduced pressure.

50 The dispersion of colour coupler 7 in aqueous gelatin was then admixed with a positive redsensitized silver chloride emulsion, which comprised per kg 75 g of gelatin and an amount of silver halide equivalent to 86 g of silver nitrate, in such an amount that after coating 1.92 g of colour coupler 7 was present per sq.m.

55 After exposure and colour-processing using 2-amino-5-diethylaminotoluene hydrochloride as colour developing agent a cyan dyestuff image having an absorption maximum of 702 nm was obtained.

#### EXAMPLE 2

60 Two positive red-sensitized silver halide emulsions were prepared as described in example 1 with the difference that instead of colour coupler 7, colour couplers 1 and 5 respectively were used. These colour couplers were incorporated into the emulsion from dispersions in aqueous gelatin, prepared as described in example 1, so that after coating on a support 1.88 g of

colour coupler 1 and 1.60 g of colour coupler 5 respectively were present per sq.m.

After exposure and colour processing using 2-amino-5-diethylaminotoluene hydrochloride as colour developing agent cyan images were obtained having absorption maxima of 696 nm and 699 nm respectively.

The cyan dyestuff images formed had a favourable resistance to heat which is clearly apparent from the table below, in which the loss in density is given of the cyan dyestuff images formed with the above colour couplers as compared with the loss in density of a cyan dyestuff image formed in a similar way using N-n-hexadecyl-1-hydroxy-4-chloro-2-naphthamide as colour coupler. The loss in density is on a percentage basis measured at density  $D = 1.5$  after storing for 24 hours at 95°C under a reduced pressure of less than 1 mm.

Table

| Dyestuff image                       | Percentage loss in density measured at density $D = 1.5$ | 20 |
|--------------------------------------|----------------------------------------------------------|----|
| Comparison dyestuff image            | -25                                                      |    |
| Dyestuff image from colour coupler 1 | -2                                                       |    |
| Dyestuff image from colour coupler 5 | -3                                                       |    |

### EXAMPLE 3

A series of three silver bromoiodide emulsions (2.3 25 mole percent of iodide) each comprising per kg an amount of silver halide equivalent to 47 g of silver nitrate and 73.4 g of gelatin was prepared.

To each of the emulsions one of the following colour couplers were added in an amount of 0.006 mole per kg : colour coupler 6, colour coupler 11 and N-n-hexadecyl-1-hydroxy-4chloro-2-naphthamide as comparison colour coupler. For this purpose the colour couplers were dissolved in ethyl acetate, the solutions formed dispersed in aqueous gelatin and the ethyl acetate removed under reduced pressure whereupon the gels obtained were admixed to the emulsions.

After dilution, adjustment of the pH and the addition of the usual additives such as hardening agents and wetting agents, the emulsions were coated on subbed cellulose triacetate supports and dried.

The materials formed were exposed for 1/20 sec. through a continuous wedge with constant 0.30 and developed for 8 min. at 20°C in a developing bath of the following composition :

|                                          |         |
|------------------------------------------|---------|
| N,N-diethyl-p-phenylene diamine sulphate | 2.75 g  |
| hydroxylamine sulphate                   | 1.2 g   |
| sodium hexametaphosphate                 | 4 g     |
| anhydrous sodium sulphite                | 2 g     |
| anhydrous potassium carbonate            | 75 g    |
| potassium bromide                        | 2.5 g   |
| water to make                            | 1000 ml |

After development the materials were treated for 2 min. at 18°-20°C in an intermediate bath comprising 30 g of sodium sulphate in 1 litre of water.

The materials were rinsed for 15 min. with water and then treated in a bleach bath of the following composition :

|                                 |         |
|---------------------------------|---------|
| borax                           | 20 g    |
| anhydrous potassium bromide     | 15 g    |
| anhydrous sodium bisulphite     | 4.2 g   |
| potassium hexacyanoferrate(III) | 100 g   |
| water to make                   | 1000 ml |

After bleaching the materials were rinsed with water for 5 min. and fixed in an aqueous solution of 200 g of sodium thiosulphate per litre.

After a final rinsing for 15 min. the materials were dried.

The cyan dyestuff images formed were then examined as to their resistance to heat as described in example 2. The results attained are listed in the following table.

5

TABLE

| Colour coupler used       | Percentage loss in density |
|---------------------------|----------------------------|
| comparison colour coupler | - 64                       |
| colour coupler 6          | - 6                        |
| colour coupler 11         | - 6                        |

We claim:

1. Photographic element comprising a light-sensitive silver halide emulsion and a colour coupler having the 15 following general formula:



wherein:

Z represents the atoms necessary to close a fused-on benzene or tetrahydrobenzene ring,

Y represents hydrogen, halogen, or sulpho in acid or salt form, azo, or  $-\text{S---R}$  wherein R stands for alkyl or aryl,

$\text{R}_1$  represents a straight-chain  $\text{C}_1\text{---C}_5$  alkyl group or an halogen-substituted aryl group,

$\text{R}_2$  represents a straight-chain  $\text{C}_1\text{---C}_5$  alkyl group, or  $\text{R}_2$  together with  $\text{R}_1$  represent the atoms necessary to close a cycloaliphatic ring, and

$\text{R}_3$  stands for a diffusion-fast making group comprising from 10 to about 20 carbon atoms in a straight alkyl chain, or  $\text{R}_3$  together with  $\text{R}_1$  represent the atoms necessary to complete a diffusion-fast making cyclo-aliphatic hydrocarbon group which comprises in the ring or together with the C-atoms of an alkyl substituent on the ring at least 12 C-atoms.

2. A photographic element according to claim 1, 45 wherein in the formula of the colour coupler  $\text{R}_3$  stands for alkyl with from 10 to about 20 C-atoms.

3. A photographic element according to claim 1, wherein in the formula of the colour coupler  $\text{R}_3$  stands for the group  $-\text{X}_1\text{---D}$  wherein D is an acyclic aliphatic 50 hydrocarbon group having from 10 to about 20 carbon atoms and  $\text{X}_1$  stands for  $-\text{COO---}$ ,  $-\text{CON}(\text{R}_4)\text{---}$ ,



60 , wherein  $\text{R}_4$  is hydrogen or  $\text{C}_1\text{---C}_5$  alkyl and  $\text{Y}_1$  is a chemical bond, oxygen, sulphur, sulphonyl,  $\text{NHCO}$ ,  $\text{CONH}$ ,  $\text{NHSO}_2$  or  $\text{SO}_2\text{NH}$ .

4. A photographic element according to claim 1, 65 wherein in the formula of the colour coupler  $\text{R}_3$  stands for the group  $-\text{CH}_2\text{---X}_2\text{---D}$  wherein D is an acyclic aliphatic hydrocarbon group having from 10 to about 20 carbon atoms and  $\text{X}_2$  stands for  $-\text{N}(\text{R}_4)\text{---}$ , sulphur,  $-\text{COO---}$ ,  $-\text{CON}(\text{R}_4)\text{---}$ ,



5  $R_4$  being hydrogen or  $C_1-C_5$  alkyl and  $Y_1$  being a chemical bond, oxygen, sulphur, sulphonyl,  $NHCO$ ,  $CONH$ ,  $NHSO_2$  or  $SO_2NH$ .

10 5. Photographic element according to claim 1 wherein said element is a multilayer colour material comprising in one of the light-sensitive silver halide emulsion layers or in a non-light-sensitive water-permeable colloid layer in water-permeable relationship with the light-sensitive silver halide emulsion layer the said colour coupler.

15 6. Process of producing a cyan dyestuff image by development of a photographic element containing imagewise exposed silver halide with the aid of a primary aromatic amino developer in the presence of a cyan-forming colour coupler corresponding to the formula:



wherein:

20  $Z$  represents the atoms necessary to close a fused-on benzene or tetrahydrobenzene ring,

$Y$  represents hydrogen, halogen, or sulpho in acid or salt form, azo, or  $-S-R$  wherein  $R$  stands for alkyl or aryl,

$R_1$  represents a straight-chain  $C_1-C_5$  alkyl group or an halogen-substituted aryl group,

$R_2$  represents a straight-chain  $C_1-C_5$  alkyl group, or

30



wherein  $R_4$  is hydrogen or  $C_1-C_5$  alkyl and  $Y_1$  is a chemical bond, oxygen, sulphur, sulphonyl,  $NHCO$ ,  $CONH$ ,  $NHSO_2$  or  $SO_2NH$ .

25 9. The process of claim 6 wherein  $R_3$  stands for the group  $-CH_2-X_2-D$  wherein  $D$  is an acyclic aliphatic hydrocarbon group having from 10 to about 20 carbon atoms and  $X_2$  stands for  $-N(R_4)-$ , sulphur,  $-COO-$ ,  $-CON(R_4)-$ ,



35  $R_4$  being hydrogen or  $C_1-C_5$  alkyl and  $Y_1$  being a chemical bond, oxygen, sulphur, sulphonyl,  $NHCO$ ,  $CONH$ ,  $NHSO_2$  or  $SO_2NH$ .

\* \* \* \* \*

40

45

50

55

60

65

$R_2$  together with  $R_1$  represent the atoms necessary to close a cycloaliphatic ring, and

$R_3$  stands for a diffusion-fast making group comprising from 10 to about 20 carbon atoms in a straight alkyl chain, or  $R_3$  together with  $R_1$  represent the atoms necessary to complete a diffusion-fast making cyclo-aliphatic hydrocarbon group which comprises in the ring or together with the C-atoms of an alkyl substituent on the ring at least 12 C-atoms.

7. The process of claim 6 wherein  $R_3$  stands for alkyl with from 10 to about 20 carbon atoms.

8. The process of claim 6 wherein  $R_3$  stands for the group  $-X_1-D$  wherein  $D$  is an acyclic aliphatic hydrocarbon group having from 10 to about 20 carbon atoms and  $X_1$  stands for  $-COO-$ ,  $-CON(R_4)-$ ,



UNITED STATES PATENT OFFICE  
CERTIFICATE OF CORRECTION

Patent No. 3,762,921 Dated October 2, 1973

Inventor(s) Hector Alfons VANDEN EYNDE ET AL

It is certified that error appears in the above-identified patent and that said Letters Patent are hereby corrected as shown below:

In the heading, [30] Foreign Application Priority Data, the priority claim should appear as follows:

-- Feb. 24, 1970      Great Britain      8839/70 --.

Column 4, lines 1 - 7, Formula 3, the formula should appear as follows:

3.



Column 5, line 52, after "Then" insert a comma (,).

Column 8, line 61, "fitered" should read -- filtered --.

Column 14, line 10, "halid" should read -- halide --.

Column 18, lines 31 - 33, claim 9, second formula, the formula should appear as follows:



Signed and sealed this 17th day of September 1974.

(SEAL)

Attest:

McCOY M. GIBSON JR.  
Attesting Officer

C. MARSHLL DANN  
Commissioner of Patents